

## UNITED STATES PATENT OFFICE

2,453,152

## CATALYTIC CONVERSION OF HYDRO-CARBONS

George Alexander Mills, Ridley Park, Pa., assignor  
to Houdry Process Corporation, Wilmington,  
Del., a corporation of Delaware

No Drawing. Application October 19, 1944,  
Serial No. 559,483

6 Claims. (Cl. 196—52)

1

The present invention relates generally to the art of the catalytic treatment of hydrocarbons and specifically to the catalytic cracking of such materials.

The application of cracking processes to crude oils, petroleum distillates and other hydrocarbon fractions has increased the amount of commercially valuable products from such sources. Various inventions concerning the apparatus and methods of conducting the fundamental process are known but only a small number of agents capable of accelerating the desired changes have been found. Industrially, the principal catalysts for cracking are certain types of activated natural clays and certain synthetic silica-alumina gel composites.

An object of the present invention is to produce fuels which improve the efficiency or power of oil engines. Another object is to crack the hydrocarbon material so that, in addition to gasoline of high anti-knock properties, the process yields by-products that can be commercially utilized. Another object is to convert hydrocarbon materials into other hydrocarbon materials more valuable in commerce by contact, under cracking conditions, with a novel catalyst. Further objects and advantages will be apparent in the following description and claims.

A preferred form of this invention is a catalytic treatment in which the hydrocarbon material to be cracked is contacted with a mass consisting essentially of colloidal silica-urania at a temperature above 700° F. under conversion conditions.

A principal application of this invention is the cracking to gasoline and valuable gaseous products, of hydrocarbon materials boiling essentially higher than gasoline. The product recovered from the contacting operation may be separated into a gaseous fraction and a synthetic crude. The synthetic crude yields, on distillation, a stable gasoline of high octane and blending value for internal combustion motors either of the automotive or aviation type. The gaseous fraction can be further processed by well-known methods of alkylation or polymerization to yield additional quantities of premium motor fuel. Selected portions of the gas may be further treated to form highly unsaturated hydrocarbons useful in the production of synthetic elastomers. The portion of the synthetic crude remaining after the removal of gasoline may be recycled to produce more gasoline or processed to yield useful products such as furnace oil, cleaners' naphtha, paint solvents or thinners, chemical intermediates and the like. However, the invention is not limited by the type

2

of charge or product and may be applied to the improvement of the stability, octane number and/or lead response of gasoline by treatment under cracking conditions; to the reforming of naphthas resulting in an increased octane number and lead response and lowered boiling ranges; to the production of fuels for oil engines not of the gasoline type; and also to the cracking of hydrocarbon gases.

10 Contact masses useful for catalytically cracking hydrocarbon materials are rare. Because of the present lack of exact knowledge concerning the actual mechanism of catalysis, the properties upon which catalytic activity depends are not known, nor has analogy with compounds showing catalytic activity proven valid in many cases. Exact predictions concerning the cracking activity of an untested combination of chemical compounds are impossible since certain combinations 15 have catalytic properties possessed by neither component and the art has not reached the stage where the effect of combining various chemical compounds can be anticipated. Therefore untested compounds or mixtures of compounds can 20 be regarded only as possible catalysts. Such conclusions must be experimentally verified.

One of the objects of this invention is to set forth an improved method of preparing a contact mass consisting essentially of colloidal silica, and 25 urania as described below. It is within the scope of the invention to use any appropriate methods of preparation such as grinding or milling mixtures of colloidal urania and colloidal silica prepared separately, reaction in the liquid or vapor state of organic compounds of uranium and silicon, impregnation of a gel of one component with the solution of a salt of the other component with subsequent decomposition of the salt, intimate mixture of hydrogels prepared separately, deposition 30 on a carrier, and the like. In all cases, a method of manufacture is used which produces a catalyst having a high specific surface, since the effectiveness of the contact mass depends on the surface. Furthermore, any method is successful only when the various components comprising the surface active mass are uniformly mixed. It is in the sense of an intimate colloidal mixture that the term "silica-urania" is used in 35 this invention. The terms, "silica," "urania" or "silica-urania," denote colloidal masses before or after calcination. "Calcination" is used in the sense of any heat treatment at a temperature above 400° F. Theories of the distinction between colloidal hydrous oxides, hydroxides, hydrated oxides and the like do not limit this invention,

nor is it limited by theories of the composition of the oxides produced on calcination.

In a preferred form of this invention, a solution of a silicate and a solution containing a compound of uranium are brought into rapid intimate contact by a mechanical mixing device under conditions whereby the hydrogels of silica and urania are concurrently formed. A third solution containing acids, alkaline compounds or neutral salts may be added simultaneously or subsequently to the solutions to adjust the pH of the final mixture, aid in pH adjustment by buffer action, or have a desired effect on the structure of the resulting hydrogel. Since the catalyst may be prepared in any form which yields aggregates of colloid size, solutions of the reagents may be treated so as to produce hydrosols, gels, gelatinous precipitates and the like as well as hydrogels. In general, the pH shown by resulting coagulum is between 2 and 11.5 but it is preferred to fix conditions so as to have an acid reaction (i. e., a pH of less than 7) shown by the resulting gels of silica and urania. Syneresis liquors may then be removed from the hydrogel, the gel dried, washed to remove salts, treated to remove adsorbed materials detrimental to the catalyst, principally alkalis, again dried, ground and formed by grinding, extrusion, pelleting or molding into convenient shapes. The sequence of operations described above is merely preferred and the invention is not limited by any specific permutation of processing operations. The finished calcined catalyst consists essentially of about 5 to 30% urania and about 95 to 70% silica. It is within the scope to add small amounts (not over 1%) of other oxides for promoter action. Thus the activity of the catalyst may be enhanced by the addition, in the original solutions or at any step in the preparation of the catalyst, of 1% or less of compounds of elements having refractory oxides such as beryllium, magnesium, zinc, strontium, barium, aluminum, titanium, zirconium, cerium, and thorium. Theoretical definitions of promoter action shall not limit the use of these minor components since the sole criterion of their effectiveness in terms of this invention is improvement in performance.

The conditions used in the process employing the prepared mass consisting essentially of colloidal silica-urania are adjusted to the type of hydrocarbon material to be converted and the degree of cracking desired. It has been found that temperatures in excess of 700° F. and below 1200° F. are suitable. In general, the space rate used will lie between 0.25 (0.25 volume of charge liquid per 1 volume of catalyst per hour) and 5. Rates in the middle portion of this range, as for instance 0.5 to 2.5, are preferred when gas oils and the like are cracked and a substantial quantity of gasoline is desired. Higher rates such as 2.0 to 5.0 are generally chosen when the operation is that of reforming a naphtha, while lower rates, such as 0.25 to 1.5, are desirable for treating cracked gasoline in order to improve its quality. The vapor pressure of the hydrocarbon material during the period of contact with the active mass may vary considerably depending on the charge and the extent and type of conversion desired. The material used as a charge to the process and catalyst described above is varied depending on the prevailing economics. Gas oil and distillates of similar boiling range are preferred when the end product is aviation gasoline. Distillates of a boiling range lower than gas oil are converted to superior motor fuels by a treatment under condi-

tions that would cause considerable cracking of a gas oil. Such distillates may be of a natural origin or may be a product from a previous cracking operation, either thermal or catalytic. Hydrocarbon mixtures containing compounds boiling higher than gas oil are cracked to give excellent yields of motor fuel when the cracking conditions are milder (lowered temperature, higher rate and/or lower cracking pressure), than those used for gas oil. Such hydrocarbon mixtures are of the type produced from the residua of crude oil distillation by such methods as tar separator distillation, coking, dewaxing, vacuum distillation, and deasphalting. Desalting and other processes which remove inorganic impurities may be used in conjunction with any of these methods. Any of the charges mentioned above may contain gasoline.

Various specific embodiments of this invention are illustrated in the following examples.

#### Example I

A solution was prepared by diluting 17.5 parts by weight of a commercial silicate (N-brand) with 163 parts by weight of water. Into this solution was poured, with agitation, a second solution containing 1 part by weight of  $UO_2(NO_3)_2 \cdot 6H_2O$  and 17 parts by weight of  $(NH_4)_2SO_4$  solution (having a specific gravity of 1.41) diluted with 92.5 parts by weight of water. A coagulum formed upon the addition of the second solution. The entire mixture had a pH of 10.0. The gel was filtered and dried in ovens at 200 to 210° F. The dried gel was washed with distilled water, then with a solution containing ammonium chloride and sufficient ammonium hydroxide to render the solution basic, finally with distilled water, and then dried in ovens at 200 to 210° F. The dry gel was ground 3 hours in a ball mill. The ground powder (1 part by weight) was mixed with 1.17 parts by weight of water and formed as pellets in a die plate. The theoretical composition of the material at this point was 90% by weight calculated as  $SiO_2$  and 10% by weight calculated as  $U_3O_8$ .

A portion of the material so prepared was heat treated for 5 hours at a temperature of 1400° F. with a mixture of 6.5% steam and 93.5% air. Some of the heat treated pellets were employed for the cracking of a gas oil essentially in accordance with the method described in detail in the "National Petroleum News" 36, No. 31, R-537-38. (Standard conditions are a space rate of 1.5, atmospheric pressure, and the temperature of the contact mass at 800° F.) The synthetic crude so produced was fractionated and yielded 6.9 volume per cent of gasoline based on the charge.

#### Example II

A solution was prepared by diluting 20.8 parts by weight of a commercial silicate (N-brand) with 9.1 parts by weight of water. A second solution was prepared by dissolving 1 part by weight of uranyl acetate in 197 parts by weight of water and adding 4.1 parts by weight of acetic acid. The two solutions were poured together with violent agitation. The theoretical composition of the hydrogel was 90% by weight calculated as  $SiO_2$  and 10% by weight calculated as  $U_3O_8$ . By the use of acetic acid and ammonium hydroxide, the final pH was adjusted to 5.6. The gel thus formed was filtered and dried in ovens at 240° F. for three hours. The dried gel was washed with distilled water, then with a solution containing ammonium chloride and finally with

distilled water. The gel was again dried and formed in a pelleting machine of the pressure type. The resulting pellets were heat treated at a temperature of 1400° F. for 10 hours in a mixture of 5% steam and 95% air.

The catalyst thus prepared was employed for the cracking of a gas oil as described in Example I, and produced 19.1 volume per cent of gasoline based on the charge. The gasoline made had a density of 0.7709 and contained 20 volume per cent of aromatics (indication of a high anti-knock value). The gas made during the cracking run showed a ratio of 8 volumes of isobutane to 1 volume of n-butane, again indicating a high anti-knock value for the gasoline produced.

I claim as my invention:

1. In the production of high octane gasoline from normally liquid hydrocarbon material by catalytic conversion processes of the type in which no hydrogen is introduced to the conversion zone, the improvement which comprises effecting said conversion by contacting said hydrocarbon material under cracking conditions including temperatures between 700° and 1200° F. with a surface active contact mass consisting essentially of silica and urania, said mass having been prepared by coprecipitation of colloidal silica and urania in an acid menstruum.

2. In the production of high octane gasoline, the process which comprises contacting normally liquid hydrocarbon material under cracking conditions with a surface active mass consisting essentially of silica and urania, said mass having been prepared by coprecipitation of colloidal silica and urania in an acid menstruum.

3. The process of claim 2 in which said surface active contact mass contains more than 5% of urania.

4. The process of claim 2 in which said surface active mass contains between 5 and 30% of urania.

5. The process which comprises cracking normally liquid hydrocarbon material comprising hydrocarbons boiling above gasoline to form substantial amounts of high octane gasoline from said hydrocarbons boiling above gasoline by contacting said hydrocarbon material under cracking

conditions with a surface active mass consisting essentially of silica and urania, said mass having been prepared by coprecipitation of colloidal silica and urania in an acid menstruum.

5. The process which comprises cracking hydrocarbon material boiling above gasoline to form substantial amounts of high octane gasoline by contacting said hydrocarbon material under cracking conditions with a surface active mass consisting essentially of silica and between 5 to 30 percent of urania, said mass having been prepared by coprecipitating colloidal aggregates of silica and urania from solutions containing soluble compounds of uranium and silicon under such conditions as to produce an acid reaction in the menstruum containing said aggregates, separating said colloidal aggregates from said menstruum, treating the separated colloidal aggregates so as to remove adsorbed materials detrimental to the catalyst and heat treating the purified colloidal aggregates at a temperature in excess of 900° F.

GEORGE ALEXANDER MILLS.

#### REFERENCES CITED

The following references are of record in the file of this patent:

#### UNITED STATES PATENTS

| Number    | Name                  | Date          |
|-----------|-----------------------|---------------|
| 1,657,753 | Jaeger et al. -----   | Jan. 31, 1928 |
| 1,870,357 | Dierichs -----        | Aug. 9, 1932  |
| 1,986,557 | Connolly et al. ----- | Jan. 1, 1935  |
| 2,258,111 | Engel -----           | Oct. 7, 1931  |
| 2,268,109 | Connolly -----        | Dec. 30, 1941 |
| 2,278,677 | Stahly et al. -----   | Apr. 7, 1942  |
| 2,291,885 | Egloff -----          | Aug. 4, 1942  |
| 2,331,338 | Michael et al. -----  | Oct. 12, 1943 |
| 2,343,192 | Kuhn -----            | Feb. 29, 1944 |
| 2,356,576 | Free et al. -----     | Aug. 22, 1944 |
| 2,370,541 | James -----           | Feb. 27, 1945 |
| 2,372,165 | Arveson -----         | Mar. 20, 1945 |
| 2,381,825 | Lee -----             | Aug. 7, 1945  |

#### FOREIGN PATENTS

| Number  | Country             | Date          |
|---------|---------------------|---------------|
| 504,614 | Great Britain ----- | Apr. 24, 1939 |